

1

3,274,014

### STABILIZED YARN COMPOSITIONS

Robert C. Harrington, Jr., and James L. Smith, Kingsport, Tenn., assignors to Eastman Kodak Company, Rochester, N.Y., a corporation of New Jersey  
No Drawing. Filed Mar. 29, 1963, Ser. No. 269,156  
9 Claims. (Cl. 106—177)

This application is a continuation-in-part of Harrington et al. U.S. patent application Serial No. 147,749, filed October 26, 1961, and now abandoned.

This invention relates to man-made fibers and fabrics made therefrom, and more particularly to such fibers and fabrics resistant to ultraviolet light.

Man-made fibers and fabrics are susceptible to degradation by ultraviolet light. For example, synthetic polymer yarn, as exemplified by cellulose ester yarn, loses both stretch and strength on exposure to light. Hence, filaments made from cellulose esters, modacrylics, polyesters, poly- $\alpha$ -olefins, halogenated synthetic resins and the like would not be used in some end products, such as window curtains or drapery linings. It therefore appears desirable to render such yarn resistant to ultraviolet light.

One object of our invention is to provide man-made fibers and fabrics which are resistant to ultraviolet light. Another object of our invention is to provide man-made filaments which are resistant to ultraviolet light. Other objects of our invention will appear herein.

We have found that yarn compositions having incorporated therein a small amount of a metal monoalkyl or monoaryl phosphate, metal dialkyl phosphate, metal alkyl phosphonate, metal alkyl (alkyl phosphonate) or metal dialkyl phosphite are resistant to ultraviolet light.

We have found zinc, chromium and aluminum salts to give best ultraviolet stabilization and of these zinc to be preferred. Preferred metal salts we have found useful in stabilizing man-made fibers and fabrics against deterioration from ultraviolet light are zinc ethyl phosphate, zinc diethyl phosphate, zinc dimethyl phosphate, zinc ethyl (ethyl phosphonate), zinc propyl phosphate, zinc ethyl phosphonate, zinc dipropyl phosphate, zinc lauryl phosphate, zinc stearyl phosphate, zinc butyl phosphate, chromium diethyl phosphate and aluminum ethyl phosphate. The ethyl derivatives are to be preferred, especially zinc ethyl phosphate.

We have found that a small amount of titanium dioxide may be used in conjunction with the phosphorus-contain-

2

ing compounds according to our invention. The preferred form of titanium dioxide is rutile.

The surprising nature of our invention is confirmed by the fact that the metal alkyl phosphates, phosphites and phosphonates used, especially the zinc compounds, themselves show no appreciable light absorption either before or after exposure to sunlight and apparently when used as yarn ultraviolet stabilizers act by some other mechanism than that of known yarn ultraviolet stabilizers, many of which are thought to act as a reducing agent or absorbers for certain portions of the light spectrum. Although we do not wish to be bound by any particular theory as to why the yarn additives of our invention are effective as ultraviolet stabilizers for 10 man-made fibers and fabrics, it may be that the metal part of the compounds exerts the sunlight-inhibiting effect.

Our invention will be further illustrated by the following examples. In these examples, yarns were spun in 20 the conventional manner, the cellulose acetate being spun from acetone solutions of a secondary cellulose acetate containing about 28% acetyl, the modacrylic from a dimethyl formamide solution, and the halogenated polymer from an acetone solution. The cellulose ester yarns, 25 all 150 denier with 38 filaments, were separately woven as filling into a 75 denier bright acetate warp. The fabric was a 5 harness satin 180 ends and 70 picks per inch. The rough or back side of the fabrics tested was about 30 80% filling. This side, which was predominately the yarn being tested, was exposed to light for different periods of time. After exposure, strips of the fabric were raveled to one inch wide strips and cut, in the direction of the filling, into 8 inch long strips. These strips were 35 pulled apart against the filling with an Instron Tensile Tester. The elongations of the strips and the pounds necessary to break the fabrics were recorded and the percent loss in strength and elongation was calculated. The test is referred to in the examples as the "ravel strip test."

#### EXAMPLE 1

Cellulose acetate yarns containing 1.4% titanium dioxide and other cellulose acetate yarns containing 1.4% titanium dioxide and 1% of various zinc salts were tested by the ravel strip test after fabrics woven therefrom had been exposed under glass to sunlight for different periods of time. The samples were inclined at a 45 degree angle to the horizon facing south. The results are listed in Table I.

Table I

| Yarn Tested                          | Langley Units of Light*  |                            |                          |                            |                          |                            |
|--------------------------------------|--------------------------|----------------------------|--------------------------|----------------------------|--------------------------|----------------------------|
|                                      | 30,000                   |                            | 70,000                   |                            | 120,000                  |                            |
|                                      | Percent Loss in Strength | Percent Loss in Elongation | Percent Loss in Strength | Percent Loss in Elongation | Percent Loss in Strength | Percent Loss in Elongation |
| Control, no stabilizer               | 12.6                     | 23.4                       | 75.0                     | 92.8                       | 84.3                     | 94.0                       |
| Zinc monoethyl phosphate, stabilizer | 0.5                      | 11.3                       | 16.7                     | 13.2                       | 24.0                     | 35.0                       |
| Zinc isopropyl phosphate             | 2.0                      | 12.3                       | 18.5                     | 15.7                       | 33.5                     | 46.3                       |
| Zinc diethyl phosphate               | 1.3                      | 10.4                       | 17.7                     | 17.8                       | 32.7                     | 44.2                       |
| Zinc ethyl phosphonate               | 6.0                      | 13.0                       | 19.5                     | 20.7                       | 41.3                     | 55.0                       |
| Zinc dipropyl phosphite              | 4.6                      | 11.2                       | 15.3                     | 15.7                       | 40.1                     | 39.7                       |
| Zinc ethyl (ethyl phosphonate)       | 5.1                      | 10.7                       | 21.2                     | 30.1                       | 50.3                     | 58.5                       |

\*10,000 Langley units of light are equivalent to exposure to Florida summer sunlight for one month under glass.

It may be seen from the above table that the incorporation of a small amount of the salts of the invention in yarn, containing a dulling pigment, reduces the loss of strength and elongation caused by exposure to sunlight.

## EXAMPLE 2

Cellulose acetate filaments containing no dulling pigment and cellulose acetate filaments containing 1% of various zinc salts of the invention were tested in the manner described in Example 1. The examples are shown in Table II.

5

|    | Sample                      | Percent Zinc Ethyl Phosphate | Percent TiO <sub>2</sub> | Langley Units (1,000)      |              |                        |                |
|----|-----------------------------|------------------------------|--------------------------|----------------------------|--------------|------------------------|----------------|
|    |                             |                              |                          | 40                         | 80           | 40                     | 80             |
|    |                             |                              |                          | Percent Loss in Elongation |              | Percent Loss in Pounds |                |
| 10 | Control 1...<br>Sample 1... | 0<br>1.0                     | 0.83<br>0.83             | 9.3<br>0.7                 | 19.7<br>17.1 | -----<br>-----         | -----<br>----- |
| 15 | Control 2...<br>Sample 2... | 0<br>1.0                     | 0<br>0                   | 87<br>78                   | 75<br>61     | -----<br>-----         | -----<br>----- |

Table II

| Yarn Tested                         | Langley Units of Light*  |                            |                          |                            |                          |                            |
|-------------------------------------|--------------------------|----------------------------|--------------------------|----------------------------|--------------------------|----------------------------|
|                                     | 30,000                   |                            | 70,000                   |                            | 120,000                  |                            |
|                                     | Percent Loss in Strength | Percent Loss in Elongation | Percent Loss in Strength | Percent Loss in Elongation | Percent Loss in Strength | Percent Loss in Elongation |
| Control, no stabilizer.....         | 7.3                      | 25.6                       | 40.2                     | 84.0                       | 78.3                     | 90.0                       |
| Zinc monoethyl phosphate.....       | 0.0                      | 14.7                       | 14.3                     | 12.7                       | 19.8                     | 30.5                       |
| Zinc diethyl phosphate.....         | 0.2                      | 11.7                       | 15.6                     | 14.5                       | 30.7                     | 40.8                       |
| Zinc ethyl phosphonate.....         | 3.0                      | 10.5                       | 17.6                     | 19.9                       | 40.2                     | 50.7                       |
| Zinc ethyl (ethyl phosphonate)..... | 4.3                      | 10.5                       | 20.7                     | 29.7                       | 50.1                     | 57.0                       |

The above Table II shows the reduction of the loss of strength and elongation of fabrics which contain a small amount of zinc alkyl phosphates and the like.

## EXAMPLE 3

Various concentrations of zinc monoethyl phosphate were incorporated in dull cellulose acetate yarn containing 1.4% TiO<sub>2</sub> to determine the effect of various concentrations of stabilizer on the rate of degradation of the filaments. The samples were exposed and tested as in Example 1, and the results are listed in the following table.

Table III

| Percent Zinc Monoethyl Phosphate in Yarn | 40,000 Langley Units of Light |                            |
|------------------------------------------|-------------------------------|----------------------------|
|                                          | Percent Loss in Strength      | Percent Loss in Elongation |
| Control, no stabilizer.....              | 15.7                          | 31.2                       |
| 1%.....                                  | 13.5                          | 20.1                       |
| 1.5%.....                                | 12.3                          | 19.4                       |
| 1.0%.....                                | 9.1                           | 10.3                       |
| 2.0%.....                                | 9.1                           | 9.2                        |

## EXAMPLE 4

Zinc monoethyl phosphate and rutile titanium dioxide were incorporated in Verel modacrylic yarn by adding to the dope from which the filaments were spun and the yarn evaluated for ability to resist degradation by exposure to Langley units of light and in a Weather-Ometer. The results are given in the following table.

40

An amount of zinc diethyl phosphite equal to 1%, based upon the polymer weight, was added to a 27% solution of a vinylidene chloride resin in acetone. The solution was exuded through small orifices into a drying chamber to produce filament yarn. The yarn was tested in a Fade-Ometer and did not show darkening or discoloration after 60 hours exposure while a control sample containing no inhibitor was darkened in 20 hours.

## EXAMPLE 6

An amount of zinc (ethyl phosphonate) equal to 1% based on polymer weight was added to a 27% acetone dope of a modified vinylidene chloride-acrylonitrile copolymer (about 50:50). Yarn spun from this dope was tested in a Fade-Ometer and showed no discoloration after 80 hours' exposure to ultraviolet light. A control containing no additive and tested under the same conditions turned brown in 20 hours.

## EXAMPLE 7

An amount of zinc bis[ethyl(ethyl phosphonate)] equal to 1% based on the polymer weight was incorporated into a 27% solids in acetone dope of a modified vinylidene chloride-acrylonitrile copolymer (about 50:50). Fibers spun from this dope were tested in a Fade-Ometer and showed no discoloration after 80 hours' exposure to ultraviolet light. A control containing no additive and tested under the same conditions turned brown in 20 hours.

## EXAMPLE 8

A number of phosphate compounds were tested for their ability to stabilize yarn against photodegradation by sunlight. Cellulose acetate was the fabric used in this instance. The results of these tests are reported in the following table.

70

75

Table V

| Sample No. | Additive <sup>1</sup>            | Fabric Properties |                        |                                                      |                                      |                        |                             |                |                        |                             |
|------------|----------------------------------|-------------------|------------------------|------------------------------------------------------|--------------------------------------|------------------------|-----------------------------|----------------|------------------------|-----------------------------|
|            |                                  | Original          |                        |                                                      | Weather-Ometer Exposure <sup>2</sup> |                        |                             |                |                        |                             |
|            |                                  | Strength, lbs.    | Percent E <sup>3</sup> | Toughness (S <sup>4</sup> × Percent E <sup>3</sup> ) | Strength, lbs.                       | Percent E <sup>3</sup> | Toughness Retained, Percent | Strength, lbs. | Percent E <sup>3</sup> | Toughness Retained, Percent |
| 78526      | 1.0% Chromium Diethyl Phosphate. | 22.7              | 23.0                   | 522.1                                                | 17.0                                 | 13.0                   | 42.3                        | 17.3           | 68                     | 22.5                        |
| 78527      | 1.0% Zinc Lauryl Phosphate.      | 25.0              | 30.0                   | 750.0                                                | 19.5                                 | 18.2                   | 47.3                        | 16.7           | 50                     | 11.1                        |
| 78528      | 1.0% Zinc Diethyl Phosphate.     | 23.3              | 28.3                   | 659.4                                                | 21.3                                 | 22.0                   | 71.1                        | 20.3           | 19.2                   | 59.0                        |
| 78529      | 1.0% Aluminum Ethyl Phosphate.   | 23.4              | 27.3                   | 638.8                                                | 19.1                                 | 18.2                   | 54.4                        | 15.1           | 6.0                    | 14.2                        |
| 78530      | 1.0% Zinc Phenyl Phosphate.      | 25.7              | 29.7                   | 763.3                                                | 18.9                                 | 16.0                   | 39.6                        | 16.8           | 10.0                   | 22.0                        |
| 78531      | 1.0% Zinc Stearyl Phosphate.     | 22.5              | 23.3                   | 524.2                                                | 15.9                                 | 5.3                    | 16.1                        | 11.0           | 3.3                    | 6.9                         |
| 78532      | 1.0% Zinc Butyl Phosphate.       | 22.4              | 31.0                   | 694.4                                                | 21.8                                 | 21.3                   | 66.9                        | 17.2           | 10.3                   | 25.5                        |
| 78612      | Control                          | 26.5              | 37.3                   | 988.4                                                | 13.3                                 | 4.3                    | 5.8                         | 13.7           | 4.0                    | 5.5                         |

<sup>1</sup> Added to cellulose acetate yarn containing 1.4% TiO<sub>2</sub>.<sup>2</sup> Weather-Ometer equipped with sunshine carbon arc.<sup>3</sup> Elongation.<sup>4</sup> Strength.

The zinc salts which we employ in accordance with our invention include the following:

(1) Zinc salts of monoalkyl, monoaryl and dialkyl acid phosphates wherein the alkyl and aryl groups include methyl, ethyl, isopropyl, n-propyl, butyl, phenyl, lauryl or stearyl.



Zinc alkyl phosphate

and



Zinc dialkyl phosphate

(2) Zinc alkyl phosphates and zinc alkyl and aryl (alkyl and aryl phosphonates) wherein the alkyl or aryl groups may be methyl, ethyl, isopropyl, n-propyl, butyl, lauryl or stearyl.



Zinc alkyl phosphonate      Zinc alkyl(alkyl phosphonate)

(3) Zinc dialkyl phosphites where the alkyl groups include methyl, ethyl, isopropyl, n-propyl, butyl, lauryl or stearyl. Preferably, the alkyl group of the zinc salts is ethyl, zinc monoethyl phosphate being particularly useful.

When metals other than zinc are used according to our invention the above formulas may be simply changed to substitute the Cr or Al or the like for the Zn and modify the structure to reflect the difference in valence.

For economic reasons, we prefer to employ about .5 to 2% of the zinc salts of the invention, based on the weight of the cellulose ester. A somewhat wider range, say 0.1 to 5%, may generally be incorporated with good results. Concentrations greater than 5% are detrimental to the properties, such as toughness, of the cellulose ester.

Representative of the cellulose esters which may be stabilized according to our invention against deterioration caused by lengthy exposure to sunlight, especially ultraviolet rays, are the lower fatty acid esters of cellulose,

e.g., cellulose acetate and triacetate, cellulose propionate, cellulose butyrate, cellulose acetate propionate, cellulose acetate butyrate; inorganic acid esters of cellulose such as cellulose nitrate; and, cellulose ethers such as ethyl cellulose.

We have found that it is advantageous in some instances to incorporate a dulling pigment in cellulosic compositions stabilized against the effects of ultraviolet light in accordance with our invention. This dulling pigment as indicated above may for example be any form of titanium dioxide, rutile titanium dioxide being especially useful.

The invention has been described in detail with particular reference to preferred embodiments thereof but it will be understood that variations and modifications can be effected within the spirit and scope of the invention as described hereinabove and as defined in the appended claims.

45 We claim:

1. A man-made filament yarn composed essentially of a fiber-forming composition selected from the group consisting of cellulose esters, acrylonitrile copolymers, polyesters and poly-alpha-olefins stabilized against deterioration from ultraviolet light containing 0.1 to 5%, based on the weight of the yarn, of a salt selected from the group consisting of (1) metal salts of monoalkyl, monoaryl and dialkyl acid phosphates; (2) metal alkyl phosphonates and metal dialkyl phosphites, said alkyl and aryl groups containing from 1 to 18 carbon atoms and said metal being selected from the group consisting of zinc, chromium and aluminum.

2. In the method of preparing cellulose acetate yarns wherein cellulose acetate is dissolved in a solvent and filaments are extruded therefrom, the step which comprises adding to the solution of cellulose acetate and solvent 0.5 to 2%, based on the weight of the cellulose acetate, of a compound selected from the group consisting of a metal monoalkyl phosphate, a metal monoaryl phosphate, a metal dialkyl phosphate, a metal alkyl phosphonate, a metal alkyl (alkyl phosphonate) and a metal dialkyl phosphite, said alkyl and aryl groups containing 1-18 carbon atoms, said metal being selected from the group consisting of zinc, chromium and aluminum, and a delustering amount of titanium dioxide.

3. Cellulose ester compositions containing .1 to 5%, base on the weight of the cellulose ester, of a compound selected from the group consisting of (1) metal salts of monoalkyl, monoaryl and dialkyl acid phosphates, (2)

metal alkyl phosphonates and metal alkyl (alkyl phosphonates), and (3) metal dialkyl phosphites, said alkyl and aryl groups containing from 1 to 18 carbon atoms and said metal being selected from the group consisting of zinc, chromium and aluminum.

4. Cellulose ester compositions containing .1 to 5%, based on the weight of the cellulose ester, of zinc monoethyl phosphate and a delustering amount of titanium dioxide.

5. Cellulose acetate compositions containing .1 to 5%, based on the weight of the cellulose acetate, of zinc monoethyl phosphate.

6. A man-made filament fabric of a yarn composed essentially of a fiber-forming composition selected from the group consisting of cellulose esters, acrylonitrile copolymers, polyesters and poly-alpha-olefins stabilized against deterioration from ultraviolet light containing 0.1-5%, based on the weight of the yarn in said fabric, of a salt selected from the group consisting of (1) metal salts of monoalkyl, monoaryl and dialkyl acid phosphates, (2) metal alkyl phosphonates and metal alkyl (alkyl phosphonates), and (3) metal dialkyl phosphites, said alkyl and aryl groups containing from 1-18 carbon atoms and

15  
10  
20

said metal being selected from the group consisting of zinc, chromium and aluminum.

7. A man-made filament fabric as defined by claim 6 wherein the fiber forming composition is a cellulosic ester.

8. A man-made filament fabric as defined by claim 6 wherein said salt is zinc monoethyl phosphate.

9. A man-made filament fabric as defined by claim 6 wherein the fiber forming composition contains from 0.1 to 5%, based on the weight of the fabric, of rutile titanium dioxide.

#### References Cited by the Examiner

##### UNITED STATES PATENTS

|           |         |                 |       |           |
|-----------|---------|-----------------|-------|-----------|
| 2,782,127 | 2/1957  | Walker et al.   | ----- | 106-177   |
| 2,825,656 | 3/1958  | Walker et al.   | ----- | 106-177   |
| 3,005,472 | 10/1961 | Kasey et al.    | ----- | 139-426   |
| 3,030,334 | 4/1962  | Canarios et al. | ----- | 260-45.75 |
| 3,052,268 | 9/1962  | Seney et al.    | ----- | 139-426   |

ALEXANDER H. BRODMERKEL, Primary Examiner.  
L. B. HAYES, Assistant Examiner.